

## UNITED STATES PATENT OFFICE.

GEORG MASING, OF BERLIN, AND OTTO DAHL, OF BERLIN-CHARLOTTENBURG, GERMANY, ASSIGNORS TO SIEMENS & HALSKE, AKTIENGESELLSCHAFT, OF SIEMENS-STADT, NEAR BERLIN, GERMANY.

## PROCESS OF IMPROVING THE QUALITIES OF NICKEL-BERYLLIUM ALLOY.

No Drawing. Application filed October 11, 1927, Serial No. 225,595, and in Germany September 16, 1928.

This invention is based upon exhaustive experiments which have shown that nickel beryllium alloys containing a preponderating amount of nickel can be manufactured and possess excellent technical properties particularly a high degree of hardness. The manufacture of the alloys may be carried out for example by melting together nickel and beryllium, or by the electrolysis of molten masses such as a mixture for example of beryllium compounds with haloids of the alkali or earth alkali metals using a nickel cathode. Thus for example it was found that an alloy containing 13.4% of beryllium is so hard that it scratches glass. A similar behavior is exhibited by the nickel beryllium alloys containing from 6 to 25% of beryllium. In general the hardness of the alloys increases with the amount of beryllium which they contain. It is, however, possible to very considerably increase the hardness of alloys which are lower in beryllium.

As an example let it be stated that alloys containing up to about 5% of beryllium can be brought to more than double their original hardness by quenching them in water or cooling them in air from a temperature in the neighborhood of or above 700° C. and afterwards heating (tempering) them to a lower temperature of about 300° to 600° C. With a beryllium content of 2½%, for example, the hardness after quenching amounts to less than 200 Brinell, after subsequent heating, however, to about 500.

The hardness can be still further increased if the alloy be suitably worked mechanically after quenching and prior to the second heating, preferably by rolling out or hammering it. In this way for example degrees of hardness of 600 Brinell and more were observed in an alloy containing about 2½% of beryllium. The rolling out of the alloy may follow the first heating.

Mechanical elongation per se is not absolutely necessary for the improvement of the alloys. Cast alloy also can be considerably increased in hardness by the above described temperature treatment. In this case the process of improvement can be modified in that when casting in chills the molten alloy is cooled in the mould instead of being quenched,

These nickel beryllium alloys can have other metals also added to them such for example as aluminium, tin, iron, cobalt, copper, etc. In such case the amount of beryllium contained in the alloy is made less and yet an improvement in the typical properties of the new alloys secured. When we speak of a nickel beryllium alloy in the specification and claims, we refer to an alloy that may or may not contain one or more additional metals.

What we claim as our invention and desire to be secured by Letters Patent is:—

1. The method for improving the qualities of a nickel beryllium alloy which contains a preponderating amount of nickel and up to 5% beryllium, consisting in heating the alloy above a temperature of approximately 700° C. and after it has cooled heating the alloy once more to a lower temperature.

2. The method for improving the qualities of a nickel beryllium alloy which contains a preponderating amount of nickel and up to 5% beryllium, consisting in heating the alloy to above 700° C. and after it has cooled, heating it at once to a temperature between 300° and 600° C.

3. A process for improving the qualities of a nickel beryllium alloy which contains a large proportion of nickel and up to about 5% of beryllium, consisting in highly heating the alloy, quenching it from above a temperature of approximately 700° C., and then reheating it to a temperature within the approximate range of 300°—600° C.

4. A method for improving the qualities of nickel beryllium alloys which contain large proportions of nickel and up to 5% beryllium, consisting in heating the alloys to a temperature above 700° C., cooling, and afterwards working them mechanically.

5. A method for improving the qualities of a nickel beryllium alloy which contains a large proportion of nickel and up to 5% beryllium, and which may contain quantities of other metals, consisting in subjecting the alloy to above a temperature of approximately 700° C., mechanically working the alloy after it has cooled and then reheating it to a lower temperature.

6. A method for improving the qualities of a nickel beryllium alloy which contains a large proportion of nickel and up to 5%

beryllium, which consists in chill casting and reheating it to a temperature within the approximate range of 300°—600° C.

7. A method for improving the qualities of a nickel beryllium alloy which contains a preponderating amount of nickel and up to 5% beryllium, consisting in heating the alloy to a temperature above 700° C., quenching it,

subjecting it to mechanical working, and reheating it to a temperature within the approximate range of 300° to 600° C.<sup>10</sup>

In testimony whereof we affix our signatures.

GEORG MASING.  
OTTO DAHL.